

May 28, 1957

J. W. TIERNEY ET AL  
PROCESS FOR MAINTAINING HIGH OXIDATION STABILITY  
IN REFINING OF LUBRICATING OILS

2,793,982

Filed Nov. 19, 1954

4 Sheets-Sheet 1



FIG. 1

INVENTORS:  
JOHN W. TIERNEY  
RICHARD E. TAYLOR  
BY

*Edward Hoban*  
ATTORNEY

May 28, 1957

J. W. TIERNEY ET AL  
PROCESS FOR MAINTAINING HIGH OXIDATION STABILITY  
IN REFINING OF LUBRICATING OILS

2,793,982

Filed Nov. 19, 1954

4 Sheets-Sheet 2



FIG. 2

INVENTORS.

BY JOHN W. TIERNEY  
RICHARD E. TAYLOR

*Edward H. Lang*  
ATTORNEY

May 28, 1957

J. W. TIERNEY ET AL  
PROCESS FOR MAINTAINING HIGH OXIDATION STABILITY  
IN REFINING OF LUBRICATING OILS

2,793,982

Filed Nov. 19, 1954

4 Sheets-Sheet 3

MODIFIED SLIGH<sup>VS</sup> OXIDATION RATE  
SULFUR CONTENT FOR NEUTRALS



INVENTOR.

BY JOHN W. TIERNEY  
RICHARD E. TAYLOR

*Edward A. Lang*  
ATTORNEY

May 28, 1957

J. W. TIERNEY ET AL  
PROCESS FOR MAINTAINING HIGH OXIDATION STABILITY  
IN REFINING OF LUBRICATING OILS

2,793,982

Filed Nov. 19, 1954

4 Sheets-Sheet 4



FIG. 4

# United States Patent Office

2,793,982

Patented May 28, 1957

1

2,793,982

## PROCESS FOR MAINTAINING HIGH OXIDATION STABILITY IN REFINING OF LUBRICATING OILS

John W. Tierney, Lafayette, Ind., and Richard E. Taylor, Woodstock, Ill., assignors to The Pure Oil Company, Chicago, Ill., a corporation of Ohio

Application November 19, 1954, Serial No. 469,989

4 Claims. (Cl. 196—24)

This invention relates to a method of preparing lubricating oil stocks having high viscosity indices with high natural oxidation resistance and pertains more particularly to an adsorption process for lubricating oil refining wherein a particular concentration range of not less than about 0.15 weight percent and not more than about 0.2 weight percent total sulfur compounds is attained for high oxidation stability and optimum flow characteristics.

It is known in the art that lubricating oil fractions of crude petroleum oils can be refined to enhance the low temperature fluidity, oxidation stability, and viscosity indices. Various refining processes have been developed including sulfuric acid treatment, adsorption, thermal diffusion, solvent extraction, extractive distillation, chemical and clay treatment to accomplish these purposes. These processes inherently remove as a chemical reaction product or solvent extract phase those non-paraffinic materials which are most unstable and deleterious to the lubricating properties of the oil. Certain of the natural sulfur, oxygen, and nitrogen compounds are also removed during these refining operations. The oxidation properties of lubricating oils are important because in service they are subjected to highly complicated oxidation atmospheres wherein oxidative reactions are catalyzed by metal surfaces and the addends present, under complex variations in temperature, pressure, oxidizing atmosphere and agitation, as the extent of use progresses. As far as the chemical structure of lubricating oils is concerned, little is known except that the aromatic content of higher boiling lubricating oil fractions (450° to 500° C.) of petroleum oils varies from 10 to 40 percent, the naphthenic content from 25 to 80 percent, and the isoparaffinic content from 15 to 75 percent, depending on the nature and source of the oil. Cyclization of the hydrocarbons has an enormous effect on viscosity while branching of the chains in acyclic hydrocarbons has little, if any, effect on viscosity. Likewise, unsaturation has little effect on viscosity in acyclic hydrocarbons although it may be an influence in cyclic compounds. A finished lubricating oil consisting as it does of these various hydrocarbons and in addition containing from 2 to 20 percent of sulfur compounds, 0.08 to 0.3 percent of nitrogen compounds and some oxygen compounds, represents a complex system for study.

It has been established, however, that although alkyl naphthenes found in white mineral oil oxidize autocatalytically and are extremely unstable as compared with straight lubricating oils, and alkyl benzenes and alkyl diphenyls are also unstable in spite of isolated instances where extremely stable hydrocarbons are found, as among the alkyl naphthalenes, the hydrocarbons in a lubricating oil are of relatively minor importance compared to organic sulfur compounds with respect to resistance to oxidation. Previous investigators have established that the natural acidic or phenolic bodies present in lubricating oils, removable by vacuum distillation from over sodium metal, are not responsible for the oxidation

2

stability of the oil and that the natural sulfur compounds seem to be the principal agents responsible for the stability of straight mineral lubricating oils. However, although refined mineral lubricating oils are generally more stable to oxidation than unrefined oils from the same source, the rate of oxidation of the former seems to speed up with use and the rate of oxidation of the latter tends to slow down with use. This may be explained in part by assuming that the rate of oxidation and sludge formation is governed by the original presence of relatively unstable compounds and is proportional to their concentration; thus, as oxidation proceeds, their concentration decreases and the increase in sludge per unit of time must also decrease. In solvent-refined oils, however, the rate of sludge formation with use increases with time. Therefore, the oxidation must be preceded by the formation of substances that oxidize easily, which reaction is accelerated by oxygen, heat and the presence of metals. In unrefined oils the rate of sludge formation decreases with time so the oxidation must be inhibited and the concentration of oxidizable substances must be slowly decreasing. Confirmation of the above and related phenomena concerning the oxidation of lubricating oils may be found in the article by Denison and Condit, 25 I. & E. Chem., 36 (11), 1945, p. 1102 and 36 (5), 1944, p. 477.

Attempts have been made to isolate the sulfur compounds naturally present in lubricating oil fractions, as by the formation of mercuric chloride addition compounds, or by selective adsorption on fuller's earth, but the results were not quantitative and the sulfur-rich extracts proved to be intractable and could not be separated or purified by ordinary chemical means. In many instances it has been reported that the sulfur-containing fractions did not inhibit the oxidation of the sulfur-free oils. The sulfur compounds themselves must be as complicated as the mixtures of hydrocarbons from which they are extracted. Research on the oxidation inhibition qualities of synthesized sulfur compounds has indicated 40 that monosulfides are good inhibitors; those sulfur compounds in which the sulfur is a part of a ring are somewhat more active, but mercaptans and disulfides are not as active on an equivalent sulfur basis as the corresponding monosulfides. These differences are partly attributed 45 to the influence of the rate of reaction of the sulfur compounds with peroxides formed or present in oil, and it is generally accepted that the rate of oxygen absorption of oils may be proportional to the peroxide concentration. Those oils which contain natural antioxidants, or agents 50 capable of reducing peroxides, will not build up high peroxide concentrations with consequent high oxidation rates. Sulfur compounds in their reaction with the peroxides are oxidized to deleterious products in the oil. The refiner, therefore, is faced with the dilemma of refining lubricating oils to improve their flow characteristics while still trying to retain a sufficient concentration of natural sulfur compounds to prevent the development of appreciable concentrations of peroxides and consequent high oxidation rates, and at the same time maintaining the content of sulfur compounds sufficiently low 55 so that upon oxidation the concentration of deleterious oxidation products is innocuous.

In accordance with the present invention it has been discovered that if lubricating oil base stocks from Mid-65 Continent crude oils, such as Van Zandt crude, are refined to a certain critical point, indicated by a total sulfur content, representing all types of sulfur compounds present, of at least about 0.15 percent by weight to about 0.2 percent by weight, there is little loss in oxidation resistance. 70 But if the sulfur content is brought below this critical level, the lubricating oil becomes highly susceptible to oxidation. In other words, a critical correlation has

been found between total sulfur content and oxidation stability for lubricating base stocks made from Mid-Continent crude oils. By maintaining the sulfur content at a level of at least about 0.15 to 0.2 weight percent, good oxidation stability of the oils is obtained. This critical level or limited range of oxidation inhibiting materials, as measured by the ultimate analysis for total sulfur content, may be produced in the lubricating oil either during refining using any of the known methods, by processing to not lower than 0.15 weight percent sulfur, or subsequent to refining by blending the phase containing the oxidation inhibiting material obtained from such refining back into the highly refined oil to attain this same critical level. Furthermore, it has been found that the concentration of the mixture of sulfur compounds, and not any particular type of natural sulfur compound is primarily responsible for the increased resistance to oxidation found above a level of about 0.15 weight percent.

Since one of the chief causes for lubricating oil deterioration is oxidation and some of the deleterious products associated with oxidation are corrosive acids, sludge, and varnish, the inhibition of which ordinarily calls for various expensive addends, it is advantageous to be able to blend or produce oils having good oxidation stability. Furthermore, the use of oxidation inhibiting addends hinges on the theory that their effectiveness is proportional to their concentrations. Since these addends are of differing effectiveness and cost, the attainment of a stable level of good oxidation resistance according to the method of this invention not only facilitates the production of highly refined, high VI base stocks with good oxidation resistance but does so economically by minimizing or eliminating the cost for anti-oxidation additives.

Accordingly, it is a primary object of this invention to provide a process for producing lubricating oil base stocks of good oxidation resistance without deleteriously affecting the other physical properties and without the need of expensive addends.

Another object of the invention is to provide a refining process wherein lubricating oil fractions and residues from Mid-Continent crude oils may be prepared by reduction of the total sulfur content to a certain critical minimum of about 0.15 weight percent, below which point the oxidation stability rapidly decreases.

Other objects and advantages of the invention will appear as the description thereof proceeds.

Figure 1 is a graph showing the oxygen absorption rate in cc./min. as abscissas plotted against the weight percent of sulfur for neutral stocks.

Figure 2 is a graph showing the oxygen adsorption in cc./min. as abscissas plotted against the weight percent of sulfur for bright stocks.

Figure 3 shows the relation between sulfur content and modified Sligh test results in mm./min. for neutral oils.

Figure 4 shows the relation between sulfur content and modified Sligh test results in mm./min. for bright stocks.

A Van Zandt crude oil having an API gravity of 33.1 was topped to remove such light fractions as gasoline, naphtha, kerosene and a light lubricating oil, leaving a topped crude having the following characteristics.

#### TOPPED CRUDE

|                    |       |
|--------------------|-------|
| Gravity ° API      | 19.7  |
| Flash ° F          | 390   |
| Pour Point ° F     | +25   |
| Vis. SUS at 210° F | 100.1 |
| Color NPA          | Black |

Boiling Range:

| Vol. percent | I. B. P. | 2.5 | 50  | 10  | 20  | 30  | 40  |
|--------------|----------|-----|-----|-----|-----|-----|-----|
| ° F          | 520      | 557 | 560 | 597 | 655 | 692 | 733 |

The above topped crude was subjected to vacuum distillation in a tower operated at a flash-zone temperature of 705° F. under absolute pressure of 90 mm. mercury with flash steam in amount of about 0.7 lb./bbl. of charge. A vacuum residue of the following characteristics was produced.

#### VACUUM RESIDUE

|                                          |       |
|------------------------------------------|-------|
| 10 Gravity ° API                         | 12.6  |
| Flash ° F                                | 575   |
| Vis. SUS @ 210° F                        | 1300  |
| Color NPA                                | Black |
| 15 Carbon residue (Conradson) percent w. | 13.5  |

The vacuum residue was deasphalting with a 6/1 propane/oil ratio in a tower having a temperature gradient of 150° to 115° F. from top to bottom and operated at 450 p. s. i. g. to produce a deasphalting oil having the following characteristics.

|                                       |      |
|---------------------------------------|------|
| 20 Gravity                            | 22.4 |
| 25 Vis. SUS @ 210° F                  | 160  |
| Color NPA                             | +6   |
| Carbon residue (Conradson) percent w. | 1.80 |

The deasphalting oil was next extracted with a 3.5/1 phenol to oil ratio in a tower having a temperature gradient of 204° F. to 192° F. from top to bottom, dewaxed to a 0° F. pour point, and contacted with 10 lbs./bbl. of clay. By control of the depth of vacuum flashing and solvent extraction, along with proper blending, there are produced an intermediate VI Bright Stock, 159 vis. @ 210° F., VI 93 and a high VI Bright Stock, 152 vis. @ 210° F., VI 99 which are more completely described in the following tables.

The vacuum distillation tower is operated to give at least three lubricating oil distillates which are separately subjected to dewaxing, solvent extraction and clay treatment to yield so called neutral stocks. By proper control of the vacuum distillation and solvent extraction steps along with proper blending there were produced two neutral stocks hereinafter identified as a 200 vis. intermediate VI neutral and a 170 vis. high VI neutral in the following tables.

Samples of each of these four lubricating oil stocks were percolated through a column of silica gel. This column was 1½ inches in diameter and 10 feet long and packed with 20-200 mesh silica gel. The gel was first wet with hexane to dissipate the high heat of wetting. About 1500 grams of each of the neutral oil stocks described above with 1500 grams of hexane were then passed through the column, followed by 1½ gallons of hexane and then 1½ gallons of benzene to completely desorb the oil on the gel. The neutral oil and solvent from the bottom of the column were collected in quart containers which were then heated in a steam bath using nitrogen stripping to remove the solvent. These neutral cuts were then combined to yield four cuts of approximately 60, 20, 10, and 10 weight percent. The 60 weight percent represented the first, or least strongly adsorbed, portion of the oil. The 20 weight percent represented that portion of the oil which was fairly strongly adsorbed, and the 10 weight percent cuts represented the most strongly adsorbed portions.

Similarly, the two bright stocks above described were subjected to percolation through fresh silica gel using higher gel-to-oil ratios than were used with the neutrals. For this operation a 3-inch diameter column 10 feet long was used and only 750 grams of each bright stock was diluted with 2250 grams of hexane. In order to obtain the 1500 grams of oil needed for testing, it was necessary to percolate two batches of each bright stock through the

column and then combine the batches. A procedure similar to that described for the neutrals was used. The complete physical properties of the individual oil stocks and the fractions or cuts obtained by silica gel treatment are given in Table I:

resinous, or very heavy compounds, shows a similar trend. It is interesting to observe that the viscosity at a given temperature increases from cut 1 to cut 4 in each instance as the aromaticity increases. This could be due to the fact that the aromatic-type compounds have higher vis-

Table I

## PROPERTIES OF VAN BASE OILS AND SILICA GEL FRACTIONS

|                      | ° API Gravity | Flash, ° F. | Fire, ° F. | Color, ASTM | RI, $n_{D}^{20}$ | Refractivity Intercept | Sulfur, Wt. percent | Neut. No. 1948 | Carbon Residue, Conradson | Viscosity, SUS |         |         | V. I. | Wt. percent of untreated Oil |
|----------------------|---------------|-------------|------------|-------------|------------------|------------------------|---------------------|----------------|---------------------------|----------------|---------|---------|-------|------------------------------|
|                      |               |             |            |             |                  |                        |                     |                |                           | 100° F.        | 130° F. | 210° F. |       |                              |
| Int. VI Neutral      | 29.4          | 430         | 465        | +2          | 1.4857           | 1.0473                 | 0.44                | 0.10           | 0.00                      | 204            | 105.2   | 46.3    | 91    |                              |
| Cut 84-1             | 32.9          |             |            | 1           | 1.4728           | 1.0440                 | 0.08                | 0.05           | 0.00                      | 164.0          | 87.3    | 44.8    | 111   | 57.6                         |
| Cut 84-2             | 30.7          |             |            | 1+          | 1.4806           | 1.0458                 | 0.17                | 0.05           | 0.00                      | 181.7          | 94.9    | 45.3    | 99    | 18.4                         |
| Cut 84-3             | 24.9          |             |            | 1/2         | 1.5014           | 1.0505                 | 0.60                | 0.05           | 0.02                      | 328            | 149.4   | 51.1    | 70    | 14.8                         |
| Cut 84-4             | 11.6          |             |            | +4/2        | 1.5577           | 1.0647                 | 3.15                | 0.05           | 0.47                      | 1831           | 512     | 73.0    | 79    | 9.2                          |
| High VI Neutral      | 31.3          | 415         | 470        | +1+         | 1.4782           | 1.0450                 | 0.18                | 0.03           | 0.00                      | 177.1          | 94.9    | 45.2    | 103   |                              |
| Cut 85-1             | 33.6          |             |            | +0          | 1.4704           | 1.0434                 | 0.05                |                | 0.00                      | 149.5          | 85.6    | 43.7    | 111   | 61.6                         |
| Cut 85-2             | 30.9          |             |            |             | 1.4800           | 1.0457                 | 0.11                |                | 0.01                      | 184.7          | 98.9    | 45.4    | 98    | 14.1                         |
| Cut 85-3             | 30.0          |             |            |             | 1.4842           | 1.0474                 | 0.19                |                | 0.00                      | 191.4          | 100.9   | 45.6    | 94    | 11.3                         |
| Cut 85-4             | 26.7          |             |            |             | 1.5060           | 1.0516                 | 1.00                |                | 0.03                      | 342            | 152.4   | 50.8    | 59    | 13.0                         |
| Int. VI Bright Stock | 24.7          | 555         | 615        | 7           | 1.4988           | 1.0473                 | 0.68                | 0.33           | 1.23                      | 2,831          | 1,019   | 159.1   | 93    |                              |
| Cut 86-1             | 29.7          |             |            | +3          | 1.4821           | 1.0446                 | 0.14                | 0.03           | 0.17                      | 1,057          | 451     | 100     | 109   | 60.4                         |
| Cut 86-2             | 10.9098       |             |            |             | 1.5047           | 1.0498                 | 0.79                | 0.03           | 2.83                      | 3,131          | 1,092   | 163.8   | 90    | 10.5                         |
| Cut 86-3             | 10.9394       |             |            |             | 1.5320           | 1.0623                 | 1.91                |                | 3.01                      | 5,660          | 1,707   | 199.4   | 69    | 14.9                         |
| Cut 86-4             | 10.9329       |             |            |             | 1.5256           | 1.0594                 | 1.72                | 0.48           | 3.60                      | 7,502          | 2,213   | 244     | 75    | 14.2                         |
| High VI Bright Stock | 26.3          | 575         | 640        | +6          | 1.4934           | 1.0450                 | 0.43                | 0.16           | 0.67                      | 2,434          | 909     | 152.1   | 99    |                              |
| Cut 87-1             | 30.0          |             |            | +2          | 1.4812           | 1.0444                 | 0.04                | 0.02           | 0.04                      | 1,243          | 517     | 107.1   | 106   | 62.3                         |
| Cut 87-2             | 24.9          |             |            |             | 1.4974           | 1.0465                 | 0.52                | 0.08           | 0.54                      | 2,517          | 941     | 167.9   | 100   | 12.6                         |
| Cut 87-3             | 19.5          |             |            |             | 1.5210           | 1.0540                 | 1.47                | 0.12           | 2.50                      | 6,434          | 1,988   | 237     | 83    | 15.9                         |
| Cut 87-4             | 19.2          |             |            |             | 1.5203           | 1.0524                 | 1.48                | 0.27           | 3.54                      | 16,135         | 4,418   | 417     | 86    | 9.2                          |

<sup>1</sup> Density at 68° F. (gm./cc.).

Referring to Table I, it is seen that as would be expected silica gel preferentially adsorbs the more polar compounds, that is, the sulfur compounds, aromatic compounds, and acidic compounds, from the fractions. There is a pronounced increase in sulfur content from cut 1 (least strongly adsorbed) to cut 4 (most strongly adsorbed) in each instance. It is to be observed that for the intermediate V. I. neutral this increase is almost 40-fold. The neutralization number, which is a measure of the acidity, follows a similar pattern.

The refractivity intercept, calculated by subtracting one-half the density at 20° C. in gm./cc. from the refractive index at 20° C. measured with sodium D light ( $n_D^{20}$ ), is a measure of the aromaticity of the cuts, higher values indicating a more aromatic material. Some typical values of the refractivity intercept for pure hydrocarbons in the lubricating oil boiling range are as follows:

- 1.0390 Double ring naphthenes
- 1.0420 Single ring naphthenes
- 1.0485 Paraffins
- 1.0620 Single ring aromatics
- 1.1000 Double ring aromatics

From the values of the refractivity intercept shown in Table I it is seen that the separation is mostly between non-aromatics, such as naphthenes, and aromatics in these lubricating oil base stocks. Thus, cut 1, run 84, has a refractivity intercept of 1.0440, which indicates primarily saturates with some aromatics. Cut 4, run 84, on the other hand, has an R. I. of 1.0647, indicating essentially all aromatics. The other cuts show a similar gradation in aromaticity from the least strongly adsorbed to the most strongly adsorbed portion. Since aromatic compounds have low viscosity indices, the V. I. would be expected to decrease from cut 1 to 4 in each instance. The carbon residue, which is an indication of the content of

cosities for the same boiling point than the naphthenes, but may also be partially explained by the tendency of silica gel to preferentially adsorb the higher molecular weight material in a homologous series.

The individual cuts of each of the oils as set forth in Table I were next blended in the following fashion. The first cut, representing about 60 percent of the oil, was used as such and called blend A. The first two cuts blended together, representing about 80 percent of the oil, were called blend B. The first three cuts blended together, representing about 90 percent of the oil, were called blend C, and all four cuts, representing 100 percent of the oil, were called blend D. In this method of blending it is to be observed that the last blend, D, in each instance should be identical with the original oil. Likewise, blend C should represent the original oil with about 10 percent of the strongly adsorbed material removed, and blend B should represent the original oil with about 20 percent of the strongly adsorbed material removed. Similarly, blend A should represent the original oil with about 40 percent of the strongly adsorbed material removed.

The blending was slightly different with the neutrals. Blend A, run 84, for example, contains all of cut 1 and enough of cut 2 to make the blend exactly 60 percent of the oil. The other blends made from the neutrals were similarly prepared. This procedure accounts for the non-fractional values under "Weight percent of untreated oils" in Table II for the neutral oils, with the exception of blend A, run 85.

Physical properties of the blends so produced are given in Table II. For the sake of convenience in following these operations, the adsorption run for the intermediate V. I. neutral is called No. 84. The run for the high V. I. neutral is called No. 85, the run for the intermediate bright stock, No. 86, and the high V. I. bright stock, No. 87.

Table II

## PROPERTIES OF BLENDS MADE FROM SILICA GEL FRACTIONS OF VAN BASE OILS

|                              | Gravity,<br>° API | Color,<br>ASTM     | RI, $n_{D}^{20}$ | Refrac-<br>tivity<br>Intercept | Sulfur,<br>Wt.<br>Percent | Neut.<br>No.<br>1948 | Carbon<br>Residue,<br>Con-<br>radson | Viscosity, SUS |         |         | Vis-<br>cosity<br>Index | Wt.<br>Percent<br>of Un-<br>treated<br>Oils |
|------------------------------|-------------------|--------------------|------------------|--------------------------------|---------------------------|----------------------|--------------------------------------|----------------|---------|---------|-------------------------|---------------------------------------------|
|                              |                   |                    |                  |                                |                           |                      |                                      | 100° F.        | 130° F. | 210° F. |                         |                                             |
| <b>Int. VI Neutral:</b>      |                   |                    |                  |                                |                           |                      |                                      |                |         |         |                         |                                             |
| Run 84—Blend A               | 32.9              | 1                  | 1.4729           | 1.0441                         | 0.07                      | 0.05                 | 0.00                                 | 161.9          | 90.4    | 44.6    | 110                     | 60.0                                        |
| Run 84—Blend B               | 32.1              | 1                  | 1.4758           | 1.0449                         | 0.11                      | 0.05                 | 0.00                                 | 172.6          | 92.6    | 45.0    | 106                     | 80.0                                        |
| Run 84—Blend C               | 31.2              | 1                  | 1.4784           | 1.0449                         | 0.15                      | 0.05                 | 0.00                                 | 180.9          | 97.6    | 45.3    | 101                     | 90.0                                        |
| Run 84—Blend D               | 29.4              | 1 <sup>1/2</sup> + | 1.4819           | 1.0435                         | 0.43                      | 0.05                 | 0.02                                 | 202            | 105.2   | 46.2    | 93                      | 100.0                                       |
| <sup>1</sup>                 | (29.4)            | (+2)               | (1.4857)         | (1.0473)                       | (0.44)                    | (0.10)               | (0.00)                               | (204)          | (105.2) | (46.3)  | (91)                    | -----                                       |
| <b>High VI Neutral:</b>      |                   |                    |                  |                                |                           |                      |                                      |                |         |         |                         |                                             |
| Run 85—Blend A               | 33.6              | 2 +16              | 1.4703           | 1.0433                         | 0.05                      | 0.05                 | 0.00                                 | 149.2          | 86.1    | 43.7    | 111                     | 61.6                                        |
| Run 85—Blend B               | 32.8              | 2 +12              | 1.4728           | 1.0438                         | 0.06                      | 0.05                 | 0.00                                 | 157.0          | 88.3    | 44.1    | 108                     | 80.0                                        |
| Run 85—Blend C               | 32.2              | 2 +17              | 1.4746           | 1.0440                         | 0.10                      | 0.05                 | 0.00                                 | 161.7          | 90.1    | 44.3    | 106                     | 90.0                                        |
| Run 85—Blend D               | 31.1              | 2 +1               | 1.4776           | 1.0438                         | 0.19                      | -----                | 0.00                                 | 172.3          | 93.3    | 44.8    | 101                     | 100.0                                       |
| <sup>1</sup>                 | (31.3)            | (1+)               | (1.4782)         | (1.0450)                       | (0.18)                    | -----                | (0.00)                               | (177.1)        | (94.9)  | (45.2)  | (103)                   | -----                                       |
| <b>Int. VI Bright Stock:</b> |                   |                    |                  |                                |                           |                      |                                      |                |         |         |                         |                                             |
| Run 86—Blend A               | 29.7              | +3                 | 1.4821           | 1.0445                         | 0.14                      | 0.03                 | 0.17                                 | 1,057          | 451     | 100.0   | 109                     | 60.4                                        |
| Run 86—Blend B               | 28.8              | +3 <sup>1/2</sup>  | 1.4854           | 1.0454                         | 0.23                      | 0.03                 | 0.21                                 | 1,206          | 503     | 107.4   | 108                     | 70.9                                        |
| Run 86—Blend C               | 27.0              | +6                 | 1.4928           | 1.0479                         | 0.51                      | 0.03                 | 0.73                                 | 1,435          | 578     | 113.5   | 102                     | 85.8                                        |
| Run 86—Blend D               | 25.4              | +7                 | 1.4976           | 1.0481                         | 0.66                      | 0.11                 | 1.17                                 | 1,730          | 667     | 123.2   | 98                      | 100.0                                       |
| <sup>1</sup>                 | (24.7)            | (7)                | (1.4988)         | (1.0473)                       | (0.68)                    | (0.33)               | (1.23)                               | (2,831)        | (1,019) | (159.1) | (93)                    | -----                                       |
| <b>High VI Bright Stock:</b> |                   |                    |                  |                                |                           |                      |                                      |                |         |         |                         |                                             |
| Run 87—Blend A               | 30.0              | +2                 | 1.4812           | 1.0444                         | 0.04                      | 0.02                 | 0.04                                 | 1,243          | 517     | 107.1   | 106                     | 62.3                                        |
| Run 87—Blend B               | 29.4              | 2                  | 1.4840           | 1.0456                         | 0.13                      | 0.02                 | 0.12                                 | 1,387          | 568     | 113.5   | 105                     | 74.9                                        |
| Run 87—Blend C               | 28.1              | +5                 | 1.4901           | 1.0482                         | 0.40                      | 0.02                 | 0.52                                 | 1,715          | 678     | 125.6   | 101                     | 90.8                                        |
| Run 87—Blend D               | 26.6              | 6                  | 1.4930           | 1.0469                         | 0.46                      | 0.04                 | 0.61                                 | 2,016          | 776     | 136.8   | 100                     | 100.0                                       |
| <sup>1</sup>                 | (26.3)            | (+6)               | (1.4934)         | (1.0450)                       | (0.43)                    | (0.16)               | (0.67)                               | (2,434)        | (909)   | (152.1) | (99)                    | -----                                       |

<sup>1</sup> Values in parentheses are properties of untreated oil from Table I.<sup>2</sup> Saybolt Colors.

In Table II, the properties of the untreated oils are listed in parentheses directly below the properties of blend D and show that in each instance blend D is practically identical with the untreated oil. This shows the accuracy of the experiments, that the silica gel has brought about no significant chemical change in the oil in the adsorption process, and that the separation is entirely physical. Obviously, the blends in Table II will show practically the same trends as the individual cuts although the changes will not be as pronounced. The agreement in the trends is very good except for the acid numbers and viscosities of the bright stock. These indicate that a very small amount of acidic, viscous material was so strongly held on the silica gel that it was not desorbed. Since the material balances in these experiments were over 99 percent, this undesorbed material represents only a very minor amount.

The various blends described in Tables I and II were then tested for oxidation stability using the oxygen absorption test. This test is conducted as follows:

A 30-gm. sample of oil is placed in a glass reaction flask, filling same to about half its height. The flask is fitted with a ground glass cover having a central oxygen delivery tube extending to within about  $1\frac{1}{2}$  inch of the bottom of the flask. As oxygen passes through the delivery tube it escapes through holes at the bottom end of the tube, mixes with the oil sample to cause a vigorous bubbling action. The oxidation of the oil liberates a certain amount of volatile hydrocarbons and acids as well as other oxidation products which are carried along with the oxygen stream through outlet tubes in the ground-glass cover or stopper leading to a water-cooled condenser. Less volatile materials condense and drop back in the flask. Unreacted oxygen and remaining contaminants leave the condenser top to enter a cold-trap immersed in a mixture of Dry Ice and methanol at a temperature below  $-100^{\circ}$  F. This trap is sufficiently cold to liquify any hydrocarbons and any acids formed during the oxidation. A pump supplies a constant flow of oxygen and the reaction flask is held at a constant tempera-

ture by a suitable bath. As oxygen is absorbed by the oil, an automatic control system operates to add oxygen from a burette by displacement of the mercury. The amount of oxygen absorbed at any specific time by the oil is indicated by the volume of mercury present in a burette. An automatic recorder connected to a leveling device draws a graph of oxygen absorbed.

Oxygen leaving the cold-trap is dried in a Drierite column and the carbon dioxide is removed by an Ascarite column. The operation of the cold-trap practically excludes any water from passing through during operation of the device but since a certain amount of water is likely to be present in the system during the set-up period (before a test is run), it is best removed as soon as possible. For further details of the construction and operation of such an oxidation apparatus reference may be made to the article entitled, "Automatic Tester for Oil Oxidation," Petroleum Processing, October 1953, page 1524. The rate of oxygen absorption in such a circulatory system is unaffected by the volatile and nonvolatile oxidation products formed. This confirms in part the results found by R. W. Dornte and C. V. Ferguson as published in their article entitled, "Oil Oxidation," Ind. Engr. Chemistry, 28(7), July, 1936, p. 863 and L. L. Davis et al., "Oxidation of Petroleum Lubricants," Ind. Engr. Chemistry, 33(3), March, 1941, page 339.

The aforesaid reference is essentially the Davis modification of the Sligh test. In the Sligh test the oxygen is bubbled through the oil at  $300^{\circ}$  F., with no catalyst present and visual examination of the amount of sludge and varnish formed is made as well as recording the rate of oxygen consumption. In the Davis modification an atmosphere of oxygen is maintained over the oil sample at  $347^{\circ}$  F. and the time required, usually about 60 minutes for a small pressure change, is noted. These results, for comparison, are corrected to 60 mm. pressure drop assuming a linear relation. The results of oxygen absorption tests are shown in Table III. For convenience, in Table III the sulfur content, neutralization number, and carbon residue of the blends are repeated.

Table III

## RESULTS OF OXYGEN ABSORPTION TESTS OF VAN BASE OILS AND BLENDED SILICA GEL FRACTIONS

| Sample Tested           | Sulfur, Wt. percent | Neut. No. 1948 | Carbon Residue, Conradson | Time, Min. | Volume Absorbed, cc. | Rate, cc./Min. | Vis. at 130° F., SUS |       |                  | Remarks                       |
|-------------------------|---------------------|----------------|---------------------------|------------|----------------------|----------------|----------------------|-------|------------------|-------------------------------|
|                         |                     |                |                           |            |                      |                | New                  | Used  | Percent Increase |                               |
| Van Int. VI Neutral     | 0.44                | 0.10           | 0.00                      | 2,880      | 225                  | 0.089          | 105.5                | 113.3 | (1)              | (1).                          |
| Van Int. VI Neutral     | 0.44                | 0.10           | 0.00                      | 2,880      | 245                  | 0.085          |                      |       | 7.4              | Slight Varnish—No Sludge.     |
| Van Int. VI Neutral     | 0.44                | 0.10           | 0.00                      | 2,880      | 120                  | 0.042          |                      |       | (1)              | (1).                          |
| Run 84—Blend A          | 0.07                | 0.05           | 0.00                      | 160        | 500                  | 3.13           | 86.2                 | 100.3 | 16.4             | Slight Varnish—No Sludge.     |
| Run 84—Blend B          | 0.11                | 0.05           | 0.00                      | 600        | 500                  | 0.833          | 93.2                 | 104.4 | 12.0             | No Varnish—No Sludge.         |
| Run 84—Blend C          | 0.15                | 0.05           | 0.00                      | 2,880      | 410                  | 0.142          | 96.8                 | 110.3 | 13.9             | Slight Varnish—Slight Sludge. |
| Run 84—Blend D          | 0.43                | 0.05           | 0.02                      | 2,880      | 155                  | 0.047          |                      |       | (1)              | (1).                          |
| Van High VI Neutral     | 0.18                | 0.03           | 0.00                      | 2,880      | 185                  | 0.064          |                      |       | (1)              | (1).                          |
| Van High VI Neutral     | 0.18                | 0.03           | 0.00                      | 2,880      | 215                  | 0.075          | 94.7                 | 99.7  | 5.3              | Slight Varnish—No Sludge.     |
| Run 85—Blend A          | 0.05                | 0.05           | 0.00                      | 110        | 500                  | 4.54           | 85.2                 | 96.0  | 12.7             | No Varnish—No Sludge.         |
| Run 85—Blend B          | 0.06                | 0.05           | 0.00                      | 138        | 500                  | 3.62           | 88.3                 | 98.6  | 11.7             | (1).                          |
| Run 85—Blend C          | 0.10                | 0.05           | 0.00                      | 1,020      | 500                  | 0.490          | 90.4                 | 99.4  | 10.0             | Slight Varnish—No Sludge.     |
| Run 85—Blend D          | 0.19                | 0.05           | 0.00                      | 2,880      | 270                  | 0.094          | 93.1                 | 99.6  | 7.0              | No Varnish—No Sludge.         |
| Van Int. VI Bright Stk. | 0.68                | 0.33           | 1.23                      | 2,880      | 150                  | 0.052          |                      |       | (1)              | (1).                          |
| Van Int. VI Bright Stk. | 0.68                | 0.33           | 1.23                      | 2,880      | 200                  | 0.069          | 1,019                | 1,105 | 8.4              | No Varnish—Slight Sludge.     |
| Run 86—Blend A          | 0.14                | 0.03           | 0.17                      | 2,880      | 300                  | 0.104          | 449.6                | 615.3 | 36.9             | No Varnish—No Sludge.         |
| Run 86—Blend B          | 0.23                | 0.03           | 0.21                      | 2,880      | 130                  | 0.045          | 505.4                | 615.8 | 21.8             | Do.                           |
| Run 86—Blend C          | 0.51                | 0.03           | 0.73                      | 2,880      | 190                  | 0.066          | 578                  | 872.2 | 42.2             | Do.                           |
| Run 86—Blend D          | 0.66                | 0.11           | 1.17                      | 2,460      | 480                  | 0.195          | 667                  | 1,149 | 72.3             | Do.                           |
| Van High VI Bright Stk. | 0.43                | 0.16           | 0.67                      | 2,880      | 135                  | 0.047          | 920.9                | 960.6 | 4.3              | No Varnish—Slight Sludge.     |
| Run 87—Blend A          | 0.04                | 0.02           | 0.04                      | 235        | 500                  | 2.13           | 517.3                | 592.0 | 14.4             | No Varnish—No Sludge.         |
| Run 87—Blend B          | 0.13                | 0.02           | 0.12                      | 1,440      | 490                  | 0.340          | 570.1                | 629.3 | 10.4             | Do.                           |
| Run 87—Blend C          | 0.40                | 0.02           | 0.52                      | 2,235      | 138                  | 0.062          | 680.4                | 783.9 | 15.2             | (1).                          |
| Run 87—Blend D          | 0.46                | 0.04           | 0.61                      | 2,880      | 175                  | 0.061          | 786.9                | 923.6 | 17.4             | (1).                          |

<sup>1</sup> These results not obtainable for 48 hour test.

For additional confirmation of the results, portions of each of the samples were subjected to the Davis modification of the Slight oxidation test. The Slight test as before mentioned measures the rate of decrease in oxygen pressure over a sample of the oil. These results are shown in Table IV.

30

stocks in Figure 2 and a sharp break in the graph again is observed at a value of about 0.15 weight percent of sulfur, below which value the oxygen absorption rate in cc./min. is excessive. The additional results plotted in Figures 3 and 4 show the rate of oxygen pressure decrease in mm./min. with decrease in sulfur content for

Table IV

## RESULTS OF SLIGH OXIDATION TESTS (DAVIS MODIFICATION)

| Oil                  | Sulphur, Wt. Percent | Temp., °F. | Time, Min. | Pressure Drop, mm.Hg | Time Corresponding to 60 mm. Pressure Drop, Minutes | Approximate of Oxidized Oil, NPA | Rate of pressure Drop, mm./min. |
|----------------------|----------------------|------------|------------|----------------------|-----------------------------------------------------|----------------------------------|---------------------------------|
| Int. VI Neutral      | 0.44                 | 347        | 307        | 61                   | 302                                                 | 6-7                              | 0.199                           |
| Run 84—Blend A       | 0.07                 | 347        | 32         | 58                   | 33                                                  | 3                                | 1.82                            |
| Run 84—Blend B       | 0.11                 | 347        | 77         | 61                   | 76                                                  | 3                                | 0.789                           |
| Run 84—Blend C       | 0.15                 | 347        | 96         | 60                   | 96                                                  | 3-4                              | 0.625                           |
| Run 84—Blend D       | 0.43                 | 347        | 274        | 62                   | 265                                                 | 5-6                              | 0.226                           |
| High VI Neutral      | 0.18                 | 347        | 160        | 60                   | 160                                                 | 5                                | 0.375                           |
| Run 85—Blend A       | 0.05                 | 347        | 17         | 62                   | 16                                                  | 2                                | 3.75                            |
| Run 85—Blend B       | 0.06                 | 347        | 35         | 65                   | 32                                                  | 2                                | 1.87                            |
| Run 85—Blend C       | 0.10                 | 347        | 88         | 52                   | 102                                                 | 3+                               | 0.588                           |
| Run 85—Blend D       | 0.19                 | 347        | 173        | 60                   | 173                                                 | 4-5                              | 0.347                           |
| Int. VI Bright Stock | 0.68                 | 347        | 246        | 60                   | 246                                                 | 8                                | 0.244                           |
| Run 86—Blend A       | 0.14                 | 347        | 108        | 60                   | 108                                                 | 5                                | 0.555                           |
| Run 86—Blend B       | 0.23                 | 347        | 156        | 60                   | 156                                                 | 5                                | 0.387                           |
| Run 86—Blend C       | 0.51                 | 347        | 168        | 60                   | 168                                                 | 8                                | 0.357                           |
| Run 86—Blend D       | 0.66                 | 347        | 92         | 60                   | 92                                                  | 8                                | 0.652                           |
| High VI Bright Stock | 0.43                 | 347        | 270        | 60                   | 270                                                 | 8                                | 0.222                           |
| Run 87—Blend A       | 0.04                 | 347        | 18         | 60                   | 18                                                  | 3-4                              | 3.33                            |
| Run 87—Blend B       | 0.13                 | 347        | 114        | 60                   | 114                                                 | 8                                | 0.526                           |
| Run 87—Blend C       | 0.40                 | 347        | 246        | 60                   | 246                                                 | 8                                | 0.244                           |
| Run 87—Blend D       | 0.46                 | 347        | 576        | 60                   | 576                                                 | 8                                | 0.104                           |

The results of these oxidation tests as given in Tables III and IV relate only to blends since the oxidation properties of the individual sulfur-rich aromatic fractions were not of primary interest. Examination of Tables III and IV shows that the untreated oils and blend D in each instance are the most stable. As sulfur and aromatic compounds are removed, the oil becomes progressively more unstable. These results are more striking when presented in graphic form and reference is therefore made to Figure 1, wherein the volume of oxygen absorption results for neutrals in cc./min. are plotted against the sulfur content. From this graph, it is apparent that as the sulfur content is reduced from about 0.45 to 0.2 weight percent, the rate of oxygen absorption slowly increases, but at a value of about 0.15 weight percent for the sulfur content, the rate of oxygen absorption suddenly and greatly increases and at any values below 0.15 weight percent of sulfur the oxygen absorption rate is excessive. Similar results are shown for the bright

neutrals and bright stocks. The results for neutrals are not quite as striking as those for bright stocks. Although the data from the modified Slight oxidation test are not quite as precise as that from the oxygen absorption test the fact that both neutrals and bright stocks of intermediate and high VI show a break at substantially the same sulfur level is significant.

To establish that the correlation found relating to the critical minimum amount of sulfur necessary to inhibit the oxidation of the lubricating oils is not related to and/or valid only for the method of treatment used herein, a 15 g. sample of the intermediate V. I. neutral was treated with 15 g. of finely divided sodium metal at about 450° F. for approximately 5 hours. This sample had a sulfur content of 0.44 weight percent before sodium treatment and after the treatment exhibited a sulfur content of 0.04 weight percent. This sodium-treated sample showed an oxygen absorption rate of 2.72 cc. per minute and exhibited a 10.6 percent viscosity increase with no

sludge or varnish. It is to be observed that this oxygen absorption rate agrees well with that obtained for the silica gel treatment shown in Figure 1, carried to the same sulfur level. Since these two methods of desulfurization are entirely different yet give comparable oxygen absorption rates at the same sulfur level with widely different aromatic contents of the treated samples, it is apparent that the content of sulfur compounds is the determining factor governing the oxygen absorption rate.

The correlation or sharp change in oxidation rate shown in the graphs at about 0.15 weight percent of sulfur could be interpreted to mean that either the type of sulfur compounds in excess of this minimum is not effective for oxidation inhibition, or there is a concentration limit above which additional amounts of the oxidation inhibiting mixture has little further effect. To determine which of these factors most accurately explains the phenomena observed, the following experiments were conducted. A sample of unstable oil (run 84, cut 1) was blended with portions of blends 2, 3, and 4 from this same intermediate V. I. neutral oil and the oxygen absorption rates and viscosity increases were observed as follows:

Table V

|               | Wt. Percent Cut 1 | Wt. Percent Sulfur of Blend | Oxygen Absorption Rate, cc./Min. | Percent Increase Viscosity |
|---------------|-------------------|-----------------------------|----------------------------------|----------------------------|
| Cuts 1+2----- | 50                | 0.11                        | 0.427                            | 12.0                       |
| Cuts 1+3----- | 90                | 0.12                        | 0.219                            | 15.6                       |
| Cuts 1+4----- | 97                | 0.15                        | 0.092                            | 5.3                        |

In making the blends shown in Table V, the relative proportions of each cut were selected so that resultant mixture would contain about 0.12 to 0.15 weight percent of sulfur. From these results it is seen that cuts 3 and 4 are at least as effective as cut 2 in reducing the oxidation rate of cut 1, and indicate that the second alternative is the predominant factor in the phenomena. Furthermore, these three points fit quite well in the curve in Figure 1, again independently confirming the phenomena and the accuracy and reliability of the experimental observations.

Another aspect of the invention is the preparation of relatively high V. I. lubricating oil compositions by blending highly refined lubricating oil base stock with sufficient amount of a concentrate of naturally-occurring, lubricating-oil-range sulfur compounds in the blend to at least about 0.15 percent w. of sulfur. For this purpose the V. I. of the lubricating oil must be not less than about 90.

Although the invention may be carried out by applying any of the known methods of physical or chemical refining or desulfurization including solvent extraction, distillation, acid treatment, adsorption, thermal diffusion and the like it is particularly adapted to adsorption techniques employing silica gel which is a commercial grade 20-200 mesh silica gel having an apparent density of 40-50 lbs./cu. ft. The refining method used to attain the results observed and claimed herein is only limited to those methods which do not chemically alter the sulfur compounds remaining in the oil. Any combination of two or more physical methods or any combination of two or more chemical methods of refining may be applied. Chemical methods and physical methods may be applied in succession to the oils treated. Since a number of chemical methods, as treatment with aqueous caustic or 2 N sodium aminoethoxide ( $H_2NC_2H_4ONa$ ) dissolved in anhydrous ethylenediamine, are specific for the removal of certain types of sulfur compounds, as the thiols, or zinc and mercury salts which are specific for cyclic sulfides, the application of these methods of refining are not preferred. However, a combination of several chemical methods in succession could be applied

to remove the various types of sulfur compounds present to the indicated level.

In addition to the foregoing considerations, the invention is particularly applicable to the mineral lubricating oil fractions obtained from Mid-Continent crude oil, especially the neutral and bright stock fractions having the physical characteristics enumerated.

The term "weight percent total sulfur" as used herein and in the claims means the percent by weight of all of the sulfur present as represented by any minor amounts of inorganic sulfur compounds present, which is usually insignificant, and the amounts of organic sulfur compounds present based on the lubricating oil.

What is claimed is:

1. The method of preparing mineral lubricating oil stocks exhibiting good resistance to oxidation comprising treating a deasphaltered, dewaxed and solvent refined lubricating oil fraction of Mid-Continent origin, containing in excess of 0.2 weight percent of total sulfur present as naturally-occurring sulfur compounds, with commercial grade 20-200 mesh silica gel having an apparent density of about 40-50 lbs./cu. ft. to reduce said sulfur content to a minimum of not less than 0.1 weight percent nor more than 0.2 weight percent based on the lubricating oil.

2. The method of preparing mineral lubricating oil stocks exhibiting good resistance to oxidation comprising, treating a deasphaltered, dewaxed, solvent refined bright stock obtained from a residual oil of Mid-Continent origin having an API gravity of about 24.7, a viscosity at 210° F. of about 159 SUS, a neutralization number of about 0.33 and containing about 0.68 weight percent of total sulfur present as naturally-occurring sulfur compounds, with 20-200 mesh silica gel at ambient temperatures to remove said sulfur compounds therefrom under conditions such that the total content of sulfur in the form of naturally occurring sulfur compounds is not less than about 0.15 weight nor more than about 0.2 weight percent based on the bright stock treated.

3. The method of preparing mineral lubricating oil stocks exhibiting good resistance to oxidation comprising, treating a deasphaltered, dewaxed, solvent refined bright stock obtained from a residual oil of Mid-Continent origin having an API gravity of about 26.3, a viscosity at 210° F. of about 152.1, a neutralization number of about 0.16, and containing about 0.43 weight percent total sulfur, with 20-200 mesh silica gel at ambient temperatures to remove said sulfur compounds therefrom under conditions such that the total content of sulfur in the form of naturally occurring sulfur compounds is not less than about 0.15 weight nor more than about 0.2 weight percent based on the bright stock treated.

4. The method of preparing mineral lubricating oil stocks exhibiting good resistance to oxidation comprising, treating a deasphaltered, dewaxed, solvent refined neutral oil obtained from the lubricating oil fractions of Mid-Continent origin having an API gravity of about 29.4°, containing about 0.44 weight percent total sulfur, having a viscosity at 100° F. of about 204 SUS and a viscosity index of about 91, with 20-200 mesh silica gel at ambient temperatures to remove said sulfur compounds therefrom under conditions such that the total content of sulfur in the form of naturally occurring sulfur compounds is not less than about 0.15 weight nor more than about 0.2 weight percent based on the neutral oil treated.

#### References Cited in the file of this patent

#### UNITED STATES PATENTS

2,404,871 Van Ess et al. ----- July 30, 1946

#### OTHER REFERENCES

Mapstone, Australian Chemical Inst. J. and Proc., vol. 14, pages 61-66, February 1947.